

# UNITED STATES PATENT OFFICE.

WINFIELD S. POTTER, OF NEW YORK, N. Y.

## PRODUCTION OF SHEETS AND PLATES OF MANGANESE STEEL.

1,017,905.

Specification of Letters Patent. Patented Feb. 20, 1912.

No Drawing.

Application filed November 3, 1911. Serial No. 658,425.

*To all whom it may concern:*

Be it known that I, WINFIELD S. POTTER, a citizen of the United States, residing in New York city, county and State of New York, have invented certain new and useful Improvements in the Production of Sheets and Plates of Manganese Steel; and I do hereby declare the following to be a full, clear, and exact description of the invention, such as will enable others skilled in the art to which it appertains to make and use the same.

My invention relates to the rolling of sheets or plates from manganese steel billets or blanks, (having a percentage of manganese above  $5\frac{1}{2}$  per cent. and usually containing about 12 per cent.) and has for its object to produce a final product of a substantially uniform fine-grained condition throughout, and having the desired stiffness or ductility appropriate to the use for which it is intended.

In carrying out my invention, I first heat the manganese steel billet or sheet bar until it is brought into a uniform and ductile condition throughout, appropriate to the rolling operation. To this end, the necessary plasticity is imparted to the billet or sheet bar by raising it to a temperature which, for the production of the best results, will usually be above the melting point of the eutectic alloy, *i. e.*, above  $1125^{\circ}$  C. (say,  $1125^{\circ}$  C. to  $1225^{\circ}$  C., according to the ductility required for rolling), but which, in some instances, may be as low as say  $1060^{\circ}$  C. provided the subsequent reduction from the billet to the sheet or plate in a single heat is not considerable. The blank is then rolled to the desired dimensions, or reheated and further rolled to gage, and if it then has a temperature above  $800^{\circ}$  C. and below  $1075^{\circ}$  C. it may be immediately quenched with the production of a product having a stiffness or ductility corresponding to the percentage of reduction and to the finishing temperature.

When the sheet cannot be finished with the intended dimensions and with the desired temperature for quenching, the rolling operation is continued until the blank has been reduced to almost its final dimensions. The rolling is then interrupted and the resulting blank is placed in a heating furnace and is therein brought to a temperature which is equalized throughout and which is sufficient to permit the continuation of the

rolling operation with the delivery of the product from the ultimate finishing pass of the rolls at a temperature between  $800^{\circ}$  C. and  $1075^{\circ}$  C. The higher temperature is preferred when greater ductility and softness are desired in the finished sheet or plate, and a lower temperature, as, for example, a temperature between  $800^{\circ}$  C. and  $900^{\circ}$  C. is preferred, when greater stiffness and a higher elastic limit in the finished product are required. At the termination of the rolling operation and preferably as soon as possible after it has issued from the last pass in the rolls, the finished sheet or plate is cooled or quenched so as to preserve the qualities due to the rolling operation as determined by the finishing temperature, together with the effects of the initial heating, which in all cases is assumed to have been such as would bring the blank to a condition of uniform solution of the constituents of the metal. After the quenching operation, the sheet may be cold rolled, which has the effect of further stiffening it and of affording smooth surfaces.

Where a lesser stiffness is required, this quality of product can be obtained by suitably reheating and quenching, and the finished sheet may be delivered to the reheating furnace direct from the rolling operation, is held therein for a short time at about the finishing temperature (say at  $800^{\circ}$  C. to  $1025^{\circ}$  C.) and is then quenched.

In the reheating operation immediately preceding the final rolling to finished gage and dimensions and particularly when in the final intended rolling operation, the percentage of reduction and the attendant compression, working and grain breakage are not sufficient alone to secure the desired hardness or stiffness, the temperature in the reheating operation should not be such nor the time of heating so long as to destroy the effects of the preceding rolling and working. In such cases, the temperature for the reheating furnace should not be much, if any, above  $1075^{\circ}$  C., nor the time during which the sheet remains in the reheating furnace more than say 12 minutes for  $\frac{1}{4}$  inch of thickness, or such time as will bring the blank to the furnace temperature throughout. Indeed, a safer limit for the temperature of the reheating operation is about  $1025^{\circ}$  C.

A tough sheet or plate of moderate stiffness may be produced by heating the blank in a temperature suitable for the required

ductility for rolling, for example, 1200° C., rolling in one or more stages and finishing above 800° C., for example, 1000° C., quenching or rapidly cooling so as to avoid loss of the wrought condition, subsequently reheating to about 1000° C., for example as hereinbefore described, and immediately quenching.

Having thus described my invention, what I claim is:

1. The method of making sheets or plates of manganese steel, which comprises heating a billet or blank of manganese steel until in a uniform and ductile condition throughout, 15 rolling and thereby working, the temperature at finishing of the working being below 1075° C. and above 800° C., and quenching; substantially as described.

2. The method of making sheets or plates 20 of manganese steel, which comprises heating a billet or blank of manganese steel until in a uniform and ductile condition throughout, rolling and thereby working, with intermediate reheating, the temperature at finishing 25 of the working being below 1075° C. and above 800° C., and quenching; substantially as described.

3. The method of making sheets or plates 30 of manganese steel, which comprises heating a billet or blank of manganese steel until in a uniform and ductile condition throughout, rolling and thereby working, the temperatures at finishing of the working being below 1075° C., and above 800° C., and 35 quenching, the quenching being preceded by reheating at about the finishing temperature, for such time only that the sheet or

plate is suitably annealed or toughened; substantially as described.

4. The method of making sheets or plates 40 of manganese steel, which comprises heating a billet or blank of manganese steel until in a uniform and ductile condition throughout, rolling and thereby working, with intermediate reheating, the temperature at finishing 45 of the working being below 1075° C., and quenching, the quenching being preceded by reheating at about the finishing temperature, for such time only that the sheet or plate is suitably annealed or toughened; 50 substantially as described.

5. The method of making sheets or plates 55 of manganese steel, which comprises heating a billet or blank of manganese steel until in a uniform and ductile condition throughout, rolling and thereby working, with intermediate reheating, the temperatures at finishing 60 of the working being below 1075° C., and quenching; substantially as described.

6. The method of making sheets or plates 65 of manganese steel, which comprises heating a billet or blank of manganese steel until in a uniform and ductile condition throughout, rolling and thereby working, with intermediate reheating to a temperature not above 1075° C., the temperature at finishing the 70 rolling being below 1075° C., and quenching, substantially as described.

In testimony whereof I affix my signature, in presence of two witnesses.

WINFIELD S. POTTER.

Witnesses:

JOHN C. PENNIE,  
MINERVA LOBEL.